

1

3,391,010  
**GOLD DECORATING COMPOSITIONS  
AND METHOD**

Anna P. Hael, West Orange, N.J., assignor to Engelhard Industries, Inc., Newark, N.J., a corporation of Delaware  
No Drawing. Filed Nov. 18, 1965, Ser. No. 508,575  
11 Claims. (Cl. 106—1)

## ABSTRACT OF THE DISCLOSURE

Process for forming gold films from gold mercaptide decorating compositions under less severe conditions than heretofore known by thermally decomposing such compositions in the presence of a halogen agent, and new improved decorating compositions for effecting such process.

This invention relates to new and improved gold decorating compositions, and is particularly concerned with gold decorating compositions which can be converted to decorative metallic gold films at temperatures substantially below those employed with compositions heretofore known in the art.

Gold decorating compositions are compositions that form a film of metallic gold when applied to various surfaces and heated. The gold compounds in such compositions have been derivatives of cyclic terpenes and sulfur, originally in the form of sulforesinates and more recently in the form of cyclic terpene mercaptides. For example, gold decorating compositions containing gold sulforesinates prepared by reacting a gold salt with a sulfurized terpene such as sulfurized Venetian turpentine have been described by Chemnitius, J. Prakt. Chem. 117, 245 (1927). Gold cyclic terpene mercaptides have been described in U.S. Patent 2,490,399.

More recently, gold decorating compositions comprising gold primary, secondary and tertiary mercaptides have been developed as described in U.S. 2,994,614, U.S. 3,163,665 and U.S. 2,984,575. Certain of these gold mercaptides, particularly the secondary and tertiary mercaptides, provide certain advantages over the previously known gold compounds used in gold decorating compositions in that relatively low temperatures are required to form a metallic film therefrom, thus extending the use of such decorating compositions to a wide range of heat-sensitive substrates such as plastics, plastic laminates, wood, paper, textiles and the like. For example, the secondary gold mercaptides of U.S. 3,163,665 can be employed to produce decorative gold coatings at temperatures as low as 145° C., and certain of the gold tertiary mercaptide decorating compositions of U.S. 2,984,575 are converted into bright, conductive gold films by heating at temperatures of 150–160° C.

While certain of the known gold mercaptide compounds employed in gold decorating compositions can be converted to gold films at relatively low firing temperatures, it must be recognized that conversion of thin films of the decorating composition to gold films may require substantial periods of time, e.g. of the order of an hour or more, and that further advantages would accrue from availability of gold decorating compositions which can be more rapidly converted to gold films at temperatures heretofore employed. Additionally, gold decorating compositions which can be fired at even lower temperatures than heretofore employed in the art would be useful, e.g. in gold coating of temperature-sensitive materials such as heat-deformable plastics and the like.

It has now been discovered that the thermal decomposition of gold decorating compositions containing organic gold mercaptide compounds can be accelerated and/or

2

effectuated at reduced temperatures by contact with a free halogen selected from the group consisting of iodine, bromine, and interhalogen compounds of iodine and bromine. The halogen agents which are used apparently destabilize the gold mercaptides so that gold films can be formed at lower temperatures. The halogen can be introduced, e.g. as vapors in a closed system, during firing. However, in a preferred embodiment of the invention, the gold formulations are mixed with the halogen just prior to application on a substrate in order to avoid undesirable destabilization of the gold solution in normal storage which would reduce the shelf life of the decorating solution. It should be understood, however, that the destabilization temperature of the halogen-containing solution will vary, depending upon the particular organic gold mercaptide compound employed, and that such solutions are within the scope of the invention.

The gold decorating solutions to which halogen agents are added according to the present invention are known per se, and generally comprise an organic gold mercaptide dissolved in a suitable organic vehicle. As hereinbefore described, such organic gold mercaptides may comprise gold resinate, cyclic terpene mercaptides, or primary, secondary or tertiary gold mercaptides of alkyl, cycloalkyl, aryl or aralkyl mercaptans. Generally speaking, the preferred mercaptans contain from one to about 20 carbon atoms in the molecule.

In addition to the gold compound, gold decorating compositions usually include a diluent therefor and may include a gold flux. The choice of diluent controls the behavior of the composition before firing and is dictated by the method by which the composition is to be applied. The diluent may be a simple solvent, but it will usually include mixtures of essential oils, terpenes, resins, and the like, carefully chosen to impart specific physical properties to the composition. These properties, such as oiliness, viscosity, evaporation rate, surface tension and tack, will vary for different methods of application. The requisite properties and the diluents required to produce them are well known to those skilled in the art of making enamels, paints and lacquers.

In addition to the diluent or solvent for the gold mercaptide, gold decorating compositions may contain a gold flux which determines the behavior of the gold film during and after firing, and is usually dictated by the composition of the article to be decorated and the use for which it is intended. The gold flux usually includes salts or resinate of bismuth, lead, boron or silicon or mixtures thereof. Salts or resinate of chromium, cadmium, tin, copper, cobalt, antimony or uranium may be employed. The gold flux improves the adherence of the gold film and its resistance to abrasion and corrosive chemicals. Other ingredients may be added to alter the color of the gold film. Silver salts and resinate, for example, give a green gold, and palladium or platinum salts or resinate give a white gold.

The halogen agent which is added to the gold decorating composition may be iodine, bromine or interhalogen compounds such as ICl, IBr, BrCl and the like. Generally, free chlorine and interhalogen compounds containing fluorine are to be avoided since they may adversely react with the containers and application equipment. The halogen agent is preferably dissolved in a solvent which is miscible with the gold decorating composition, e.g., ether, chloroform or the like, and the solution of halogen agent added to provide from about 1% to about 100% by weight, of halogen agent, based on the weight of gold in the mixture.

As mentioned hereinbefore, the addition of the halogen agent to the gold decorating composition lowers the temperature at which the gold mercaptide can be converted to metallic gold. While the halogen agent can

3

be added in certain instances to the gold decorating composition to provide the novel compositions of the invention, it is preferable to make the addition shortly before use of the gold decorating composition. Using the method of this invention, gold films can be formed at temperatures as low as 80° to 90° C., and when employed at more elevated temperatures, the halogen-containing gold decorating solutions of the invention are converted more rapidly to gold films than are similar solutions which do not contain free halogen.

### EXAMPLE 1

A gold decorating solution containing 1.87% by weight gold was prepared by admixing the following (all percentages by weight):

|                                                                                       | Percent |
|---------------------------------------------------------------------------------------|---------|
| Ether                                                                                 | 78.15   |
| Gold t-dodecyl mercaptide solution in n-heptane<br>and chloroform containing 28% gold | 6.65    |
| n-Hexanol                                                                             | 4.00    |
| IBr in chloroform (10%)                                                               | 11.20   |

The gold solution was sprayed on a thin (0.03" thick) sheet of cellulose acetate and heated by means of an infrared lamp held about 5½ inches from the sample. A gold coating with a highly reflective surface was developed in 5–10 minutes, and the temperature-sensitive substrate (deformation temperature 100°C.) was not deformed. Similar films were developed on this substrate in constant temperature ovens at 80–90°C.

**EXAMPLE 2**

A gold solution containing 3.75% by weight gold was prepared by admixing the following:

|                                                                                       | Percent |
|---------------------------------------------------------------------------------------|---------|
| Ether                                                                                 | 66.10   |
| Gold t-dodecyl mercaptide solution in n-heptane<br>and chloroform containing 28% gold | 13.35   |
| Oil of peppermint                                                                     | 4.00    |
| IBr in chloroform (10%)                                                               | 16.55   |

Thin sheets of cellulose acetate were immersed in this solution and heated at 80-90° C. to produce highly reflective gold films.

## EXAMPLE 3

The following gold solution containing 2% gold was sprayed on a thin sheet of cellulose acetate:

|                                                                                       | Percent |
|---------------------------------------------------------------------------------------|---------|
| 5 Oil of peppermint                                                                   | 6.25    |
| Gold t-dodecyl mercaptide solution in n-heptane<br>and chloroform containing 28% gold | 7.13    |
| Chloroform                                                                            | 86.62   |

10 The coated substrate was exposed to radiation from a 250 watt infrared lamp at a distance of 8 inches. After 10 minutes, a dark film having some metallic appearance, but containing large iridescent purple areas, resulted. This film had only slight electrical conductivity, 15 indicating that considerable organic matter was present in the film. Further heating under the same conditions resulted in extreme deformation of the substrate without significant improvement in the film.

**EXAMPLE 4**

A gold solution containing 1.87% by weight gold was prepared from the following:

|                                                                                       | Percent |
|---------------------------------------------------------------------------------------|---------|
| IBr in chloroform (solution of 10%)                                                   | 1.35    |
| I <sub>2</sub> in chloroform (solution of 2.6%)                                       | 0.64    |
| Ether                                                                                 | 87.36   |
| Oil of peppermint                                                                     | 4.00    |
| Gold t-dodecyl mercaptide solution in n-heptane<br>and chloroform containing 28% gold | 6.65    |

30 This solution was sprayed on a thin sheet of cellulose acetate and heated in an oven at 80° C. for 1½ hours. A highly reflective gold film was formed on the substrate.

### EXAMPLES 5-18

35 A series of gold decorating solutions containing various organic gold mercaptides was prepared and tested for their ability to deposit a decorative metallic gold film. In each case, the solutions were applied to either a thin cellulose acetate sheet or, for higher temperature trials  
40 to glazed porcelain and the coated substrate placed in a preheated oven at the indicated temperature for the time period indicated. The composition of the solutions and the results are shown in the following table.

| Example | Composition                                     | Weight Percent | Temp., ° C. | Time (Hrs.) | Quality of Film          |
|---------|-------------------------------------------------|----------------|-------------|-------------|--------------------------|
| 5.      | Gold-2-pinanyl mercaptide.....                  | 6.0            | 120         | 2.5         | No gold deposit.         |
|         | Benzene.....                                    | 90.0           |             |             |                          |
|         | Oil of peppermint.....                          | 4.0            |             |             |                          |
|         | (Total gold 2.4%)                               |                |             |             |                          |
| 6.      | Solution of Example 5.....                      | 87.0           | 120         | 2.5         | Bright gold, conductive. |
|         | IBr.....                                        | 0.13           |             |             |                          |
|         | Chloroform.....                                 | 12.87          |             |             |                          |
|         | (Total gold 2.1%)                               |                |             |             |                          |
|         | Gold diphenylmethyl mercaptide.....             | 4.0            | 150         | 2.5         | No gold deposit.         |
|         | Toluene.....                                    | 50.0           | 300         | 1           | Do.                      |
| 7.      | Ether.....                                      | 40.0           | 400         | 1           | Bright gold, conductive. |
|         | Oil of peppermint.....                          | 6.0            |             |             |                          |
|         | (Total gold 1.9%)                               |                |             |             |                          |
|         | Gold diphenylmethyl mercaptide.....             | 4.0            |             |             | Bright gold.             |
|         | Ether.....                                      | 40.0           | 150         | 2.5         |                          |
| 8.      | Chloroform.....                                 | 47.97          |             |             |                          |
|         | Oil of peppermint.....                          | 6.0            |             |             |                          |
|         | I.....                                          | .63            |             |             |                          |
|         | IBr.....                                        | 1.40           |             |             |                          |
|         | (Total gold 1.9%)                               |                |             |             |                          |
|         | Gold-1-methyldodecyl mercaptide in toluene..... | 8.0            | 120         | 1           | No gold deposit.         |
|         | Ether.....                                      | 50.0           | 150         | 1           | Do.                      |
| 9.      | Chloroform.....                                 | 38.0           |             |             |                          |
|         | Oil of peppermint.....                          | 4.0            |             |             |                          |
|         | (Total gold 2.2%)                               |                |             |             |                          |
| 10.     | Solution of Example 9.....                      | 87.00          | 120         | 1           | Bright gold, conductive. |
|         | IBr.....                                        | .13            | 150         | ½           | Do.                      |
|         | Chloroform.....                                 | 12.87          |             |             |                          |
|         | (Total gold 1.9%)                               |                |             |             |                          |
|         | Gold-p-tert-butyl phenyl mercaptide.....        | 6.0            | 150         | 1           | No gold deposit.         |
| 11.     | Ether.....                                      | 50.0           |             |             |                          |
|         | Chloroform.....                                 | 40.0           |             |             |                          |
|         | Oil of peppermint.....                          | 4.0            |             |             |                          |
|         | (Total gold 3.3%)                               |                |             |             |                          |
|         | Solution of Example 11.....                     | 87.00          | 120         | 1           | Bright gold, conductive. |
| 12.     | IBr.....                                        | .13            | 150         | 1           | Do.                      |
|         | Chloroform.....                                 | 12.87          |             |             |                          |
|         | (Total gold 2.9%)                               |                |             |             |                          |
|         | Gold-tert-tetradecyl mercaptide.....            | 6.0            | 150         | 1           | No gold deposit.         |
|         | Ether.....                                      | 50.0           | 300         | 1           | Bright gold, conductive. |
| 13.     | Chloroform.....                                 | 40.0           |             |             |                          |
|         | Oil of peppermint.....                          | 4.0            |             |             |                          |
|         | (Total gold 2.6%)                               |                |             |             |                          |

| Example | Composition                                                                                                                       | Weight Percent                               | Temp., ° C.              | Time (Hrs.)      | Quality of Film                                                                                   |
|---------|-----------------------------------------------------------------------------------------------------------------------------------|----------------------------------------------|--------------------------|------------------|---------------------------------------------------------------------------------------------------|
| 14.     | Solution of Example 13.....<br>IBr.....<br>Chloroform.....<br>(Total gold 2.3%)<br>Gold-tert.-nonyl mercaptide.....<br>Ether..... | 87.00<br>.13<br>12.87<br>7.5<br>50.0<br>37.5 | 120<br>150<br>150<br>300 | 1<br>1<br>1<br>1 | Bright gold, not conductive.<br>Bright gold, conductive.<br>No gold deposit.<br>Gold, conductive. |
| 15.     | Chloroform.....<br>Oil of peppermint.....<br>(Total gold 4.0%)<br>Solution of Example 15.....<br>IBr.....                         | 5.0<br>87.00<br>.13<br>12.87                 | 150                      | 1                | Bright gold, conductive.                                                                          |
| 16.     | Chloroform.....<br>(Total gold 3.5%)<br>Gold alpha-methylbenzyl mercaptide.....<br>Benzene.....                                   | 4.0<br>90.0<br>6.0                           | 120<br>150               | 1<br>1           | No gold deposit.<br>Do.                                                                           |
| 17.     | Oil of peppermint.....<br>(Total gold 2.0%)<br>Solution of Example 17.....<br>IBr.....                                            | 87.00<br>.13<br>12.87                        | 120<br>150               | 1<br>1           | No gold deposit.<br>Bright gold, conductive.                                                      |
| 18.     | Chloroform.....<br>(Total gold 1.7%)                                                                                              |                                              |                          |                  |                                                                                                   |

The results shown in the table demonstrate that gold 20  
decorating compositions containing various gold mer-  
captide compounds are converted, in the presence of  
added halogen, to bright conductive gold films more  
rapidly and at substantially lower temperatures than are  
effective in the absence of the halogen agent.

What is claimed is:

1. A gold decorating composition comprising an organic gold mercaptide dissolved in an organic vehicle, said gold mercaptide being selected from the group consisting of gold resinates, cyclic terpene mercaptides, and primary, secondary, and tertiary gold mercaptides of alkyl, cycloalkyl, aryl, and aralkyl mercaptans containing from 1 to about 20 carbon atoms in the molecule, and said composition containing from about 1% to about 100% by weight, based on the weight of gold, of a free halogen selected from the group consisting of iodine, bromine and interhalogen compounds of iodine and bro-

mine.

2. Composition of claim 1 wherein the organic gold mercaptide is a gold terpene mercaptide.

3. Composition of claim 2 wherein the organic gold mercaptide is gold 2-pinanyl mercaptide.

4. Composition of claim 1 wherein the organic gold mercaptide is a tertiary alkyl mercaptide having up to 20 carbon atoms in the molecule.

5. Composition of claim 4 wherein the tertiary mer-  
captide is t-dodecyl gold mercaptide.

6. Composition of claim 4 wherein the gold mercap-  
tide is t-nonyl gold mercaptide.

7. Composition of claim 4 wherein the gold mercap-  
tide is t-tetradecyl gold mercaptide.

8. Composition of claim 1 wherein the organic gold mercaptide is a gold secondary alkyl mercaptide having up to 20 carbon atoms in the molecule.

9. Composition of claim 1 wherein the organic gold mercaptide is a gold aryl mercaptide having up to 20 carbon atoms in the molecule.

10. In the method for forming a decorative gold film by coating a substrate with a gold decorating composition containing an organic gold mercaptide selected from the group consisting of gold resinates, cyclic terpene mercaptides, and primary, secondary, and tertiary gold mercaptides of alkyl, cycloalkyl, aryl, and aralkyl mercaptans containing from 1 to about 20 carbon atoms in the molecule, and heating the coated substrate to thermally decompose the gold compound to metallic gold, the improvement of effecting said thermal decomposition of the gold compound in contact with a free halogen selected from the group consisting of iodine, bromine and interhalogen compounds of iodine and bromine.

11. In the method for forming a decorative gold film by coating a substrate with gold decorating composition containing an organic gold mercaptide selected from the group consisting of gold resinates, cyclic terpene mercaptides, and primary, secondary, and tertiary gold mercaptides of alkyl, cycloalkyl, aryl, and aralkyl mercaptans containing from 1 to about 20 carbon atoms in the molecule, and heating the coated substrate to thermally decompose the gold compound to metallic gold, the improvement of adding to the gold decorating composition prior to use thereof of a free halogen selected from the group consisting of iodine, bromine and interhalogen compounds of iodine and bromine, such free halogen being added in the amount of 1% to about 100% by weight of halogen based on the weight of gold.

#### References Cited

##### UNITED STATES PATENTS

|           |        |                |       |
|-----------|--------|----------------|-------|
| 2,984,575 | 5/1961 | Fitch          | 106—1 |
| 2,994,614 | 8/1961 | Fitch          | 106—1 |
| 3,092,504 | 6/1963 | Langley et al. | 106—1 |
| 3,245,809 | 4/1966 | Fitch          | 106—1 |

JAMES A. SEIDLECK, Primary Examiner.

L. B. HAYES, Assistant Examiner.